

# United States Patent

[19]

Harris et al.

[11] 3,926,550

[45] Dec. 16, 1975

[54] **COTTON-TUNG OIL DURABLE-PRESS  
TEXTILES WITH HIGH FLEX ABRASION  
RESISTANCE**

[75] Inventors: **James A. Harris**, Pearl River; **Jett C. Arthur, Jr.**, Metairie, both of La.

[73] Assignee: **The United States of America as  
represented by the Secretary of  
Agriculture**, Washington, D.C.

[22] Filed: **Nov. 26, 1974**

[21] Appl. No.: **527,399**

[52] **U.S. Cl.** ..... **8/116 R**; 8/115.6; 8/193;  
8/194; 106/252; 204/159.12; 260/23 CP;  
260/23 ST; 427/36; 427/352; 427/382;  
427/392

[51] **Int. Cl.<sup>2</sup>** ..... **D06M 13/02**; D06M 13/20

[58] **Field of Search** ..... 427/308, 392, 36; 106/252;  
8/115.6, 116 R, 193, 194

## [56] References Cited

### UNITED STATES PATENTS

1,699,779 1/1929 Cochran ..... 8/115.6

|           |         |                    |         |
|-----------|---------|--------------------|---------|
| 1,984,139 | 12/1934 | Koch.....          | 106/252 |
| 2,381,653 | 8/1945  | Drummond.....      | 106/252 |
| 2,890,137 | 6/1959  | Vaughan et al..... | 427/392 |
| 3,101,276 | 8/1963  | Hendricks.....     | 427/308 |
| 3,488,210 | 1/1970  | Kuzmak et al.....  | 8/116 R |
| 3,514,385 | 5/1970  | Magat et al.....   | 8/193   |

*Primary Examiner*—Murray Tillman

*Assistant Examiner*—Arthur H. Koeckert

*Attorney, Agent, or Firm*—M. Howard Silverstein; Max D. Hensley

[57]

## ABSTRACT

Cotton fabric is impregnated with one of several organic solutions containing tung oil and subjected to either a high-energy radiation treatment or to a specific heat treatment, thus initiating a reaction with the cellulose which yields a cotton fabric with durable-press properties. Of special interest is the unusually high flex abrasion resistance obtained.

13 Claims, No Drawings

## COTTON-TUNG OIL DURABLE-PRESS TEXTILES WITH HIGH FLEX ABRASION RESISTANCE

This invention relates to a process for chemically treating cotton fabrics. More specifically, this invention relates to the impregnation of cotton fabric with a naturally occurring product to improve its physical properties. Cotton fabric is impregnated with tung oil, which is obtained from the fruit of the tree *Aleurites fordii*, and then subjected to a high energy radiation treatment and/or a heat treatment to yield a cotton textile with durable-press properties, such as improved wrinkle recovery after deformation and improved flex abrasion resistance, thereby increasing the utility of cotton textile products in markets requiring easy care properties.

The actual processing can be described in a plural manner to yield at least three processes, thusly:

1. Solutions of tung oil in organic solvents, such as acetone, N,N-dimethylformamide, methyl ethyl ketone, and petroleum ether, are padded onto cotton textile fabrics. The physical properties of these treated cotton textile fabrics are permanently modified by thermally and/or high energy radiation initiated oxidative polymerization of the added tung oil to yield textile products with durable-press properties.

2. Solutions of tung oil in organic solvents, such as acetone, N,N-dimethylformamide, methyl ethyl ketone, and petroleum ether, containing vinyl monomers, such as acrylonitrile, 1,3-butylene dimethacrylate, diacetone acrylamide, glycidyl methacrylate, or styrene, are padded onto cotton textile fabrics. The physical properties of the treated cotton textile fabrics are permanently modified by thermally and/or high energy radiation initiated polymerization of the added tung oil and vinyl monomer to yield textile products with durable-press properties.

3. Solutions of tung oil in organic solvents, such as acetone, N,N-dimethylformamide, methyl ethyl ketone, and petroleum ether, are padded onto cotton textile fabrics, then cellulosic crosslinking reagents are padded onto the tung oil treated cotton textile fabrics either before or after the oxidative polymerization of the tung oil has been thermally initiated, and finally thermally curing the tung oil treated cotton textile fabrics containing cellulosic crosslinking reagents to yield textile products with durable-press properties.

The process of this invention has as its objective the modification of the morphological structures of cotton textile fabrics by deposition of chemical reagents in solution within the morphological structures of the fabrics and then oxidatively polymerizing said chemical reagents within the morphological structures of the fabrics by thermal and/or high energy radiation initiation. Thereby a cotton textile fabric product is prepared which has durable-press properties, particularly retention and recovery of initial shape after deformation, that is wrinkle recovery and flex abrasion resistance, so that durable-press cotton textile products with easy care properties are obtained.

Developments in the commercial use of durable-press textiles have generally led to the use of blends of cotton fibers and man-made chemical fibers in order to have products with easy care properties with minimum losses of the natural properties of cotton. When all-cotton fabrics are finished by normally used processes in which selected reagents are cured with chemical catalysts at high temperatures on the fabrics, usually drastic losses in the natural properties of the cotton fabrics

occur. We have discovered that a naturally occurring chemical, tung oil, can be padded onto cotton fabrics to yield all-cotton textiles with durable-press properties. Tung oil, obtained from the fruit of the tree *Aleurites fordii* grown in the southern area of the United States of America and other countries, is a glycerine derivative of stearic acid with about 75 percent of the acid composed of eleostearic acid, which contains three conjugated double bonds, while padded onto cotton textile fabrics can be oxidatively polymerized by thermal and/or high energy radiation initiation. We found that this oxidative polymerization of the tung oil leads to changes in the morphological structures of the cotton textile fabrics and in the physical properties of the tung oil modified fabrics to impart durable-press properties to the cotton textile fabrics.

We have now discovered that when tung oil from solutions of organic solvents, such as acetone, N,N-dimethylformamide, methyl ethyl ketone, and petroleum ether, are padded onto cotton textile fabrics to add-ons of tung oil ranging from 10 to 29 percent and cured at temperatures ranging from 200° to 300° F at times ranging from 2 to 8 minutes and/or irradiated at ambient temperatures (about 77°F) by cobalt-60 gamma-radiation to dosages ranging from 1 to 2.3 megarads, durable-press cotton textile products with improved properties over those of durable-press cotton textile products prepared by the usual thermally and chemically catalyzed crosslinking processes. We have further discovered that if vinyl monomers, such as acrylonitrile, 1,3-butylene dimethacrylate, diacetone acrylamide, glycidyl methacrylate, or styrene are added to the solutions of tung oil in ratios ranging from 1 part of tung oil and 1 part of vinyl monomer to 7 parts of tung oil and 1 part of vinyl monomer prior to the padding and subsequent processing steps, durable-press cotton textile products with improved properties over those of durable-press cotton textile products prepared by the usual thermally and chemically catalyzed crosslinking processes. Further, we have found that the usual crosslinking chemical reagents, without the addition of chemical catalysts, which are primarily responsible for the drastic losses in the desirable natural properties of cotton fabrics, may be combined with the tung oil treatment of cotton fabrics either prior to or after oxidative polymerization of the tung oil within the cotton fabric structure to yield durable-press cotton textile products with improved properties over those of cotton textile products prepared by the usual processes.

The following examples are provided to illustrate the invention and are not to be construed as limits to the invention in any manner whatsoever.

### EXAMPLE 1

#### Heat Curing and Add-on Study

Cotton fabric (printcloth about 3.4 oz/yd<sup>2</sup>), which had been enzymatically desized, alkali scoured, peroxide bleached, and dried to normal regain moisture content was immersed in about 30 percent solution of tung oil in N,N-dimethylformamide for 2 hours or more at 77°F until the cotton fabric was thoroughly wetted with the solution; then the cotton fabric was padded to the desired wet pickup of about 80-120%. The tung oil treated cotton fabric was dried for 3 minutes at about 140°F in an air oven.

The six samples of the dried, tung oil-treated cotton fabric were cured for different times at different tem-

peratures (see Table 1, samples 4-9, and controls 1-3). Selected durable-press properties of these cured, tung oil treated fabrics were compared with those of untreated cotton fabric, heated untreated cotton fabric, and cotton fabric crosslinked with dimethyloldihydroxyethylene urea (DMDHEU) and cured with chemical catalysts at 320°F for 6 minutes in accordance with prior art. DMDHEU add-on was 8%. The selected durable-press properties of the fabrics were determined in accordance with methods of the American Society for Testing and Materials, Philadelphia, Pa., as follows: (1) tear strength, ASTM method D 1424-63; (2) flex abrasion resistance, ASTM method D 1175-64T; and (3) wrinkle recovery angle, ASTM D 1295-60T. The selected durable-press properties of the fabrics are tabulated below (see Table 1).

ded, and dried (using the method of Example 1). Then samples of the dried, tung oil treated cotton fabric were cured at 300°F for 6 minutes. Then these cured, tung oil treated fabrics were extracted with selected organic solvents and dried. Then selected durable-press properties of the fabrics were determined and are tabulated below. The control fabrics were the same as those in Example 1. The tung oil treated fabrics, which had been immersed in solutions of tung oil and N,N-dimethylformamide and, after curing, extracted with methyl ethyl ketone had wrinkle recovery angle of 260°, tear strength of 493 grams, and flex abrasion resistance of 976 cycles which were improved selected durable-press properties, as compared with other tung oil treated fabrics and fabrics cross-linked by the method of prior art, as examination of data in Examples 1 and 2 show

TABLE I

Effects of Temperature and Time of Curing on the Properties of Tung Oil - Cotton Fabrics

| Sample No.       | Temp. °F | Time min. | Tung Oil Add-On % | Tear Strength grams | Flex Abrasion Resistance, cycles | Wrinkle Recovery Angle-Wet, degrees |
|------------------|----------|-----------|-------------------|---------------------|----------------------------------|-------------------------------------|
| Control Fabrics  |          |           |                   |                     |                                  |                                     |
| 1                | —        | —         | —                 | 820                 | 713                              | 195                                 |
| 2                | 300      | 6         | —                 | 720                 | 391                              | 168                                 |
| 3                | 320      | 6         | (a)               | 207                 | 13                               | 277                                 |
| Research Fabrics |          |           |                   |                     |                                  |                                     |
| 4                | 300      | 2         | 10                | 500                 | 286                              | 207                                 |
| 5                | 300      | 4         | 17                | 460                 | 376                              | 251                                 |
| 6                | 300      | 6         | 22                | 413                 | 449                              | 247                                 |
| 7                | 300      | 8         | 23                | 353                 | 395                              | 251                                 |
| 8                | 200      | 6         | 29                | 400                 | 575                              | 245                                 |
| 9                | 250      | 6         | 27                | 453                 | 546                              | 252                                 |

(a) Dimethyloldihydroxyethylene urea add-on 8 percent by method of prior art.

The tung oil treated cotton fabrics, which contained (see Table II).

TABLE II

Effects of Solvent Used to Prepare Solution of Tung Oil on the Properties of Tung Oil Cotton Fabrics

| Sample No. | Solvent Immersion | Used <sup>a</sup> Extraction | Tung Oil Add-on, % | Tear Strength, grams | Flex Abrasion Resistance, cycles | Wrinkle Recovery Angle-Wet, degrees |
|------------|-------------------|------------------------------|--------------------|----------------------|----------------------------------|-------------------------------------|
| 10         | MEK               | MEK                          | 27                 | 350                  | 200                              | 234                                 |
| 11         | DMF               | MEK-DMF                      | 22                 | 413                  | 449                              | 247                                 |
| 12         | DMF               | MEK                          | 18                 | 493                  | 976                              | 260                                 |
| 13         | DMF-PE            | DMF                          | 27                 | 420                  | 628                              | 261                                 |
| 14         | DMF-A             | MEK                          | 26                 | 380                  | 525                              | 241                                 |

<sup>a</sup> MEK, methyl ethyl ketone; DMF, N,N-dimethylformamide; PE, petroleum ether; A, acetone; MEK-DMF, equal parts; DMF-PE, equal parts; DMF-A, equal parts.

17% to 29% tung oil had wrinkle recovery angles of 55 245°-252°, tear strengths of 353-460 grams, and flex abrasion resistances of 376-575 cycles, as compared with fabric crosslinked by the method of the prior art of 277°, 207 grams, and 13 cycles. The data conclusively indicate that the tung oil treated cotton fabrics had better durable-press properties that were measured than control fabrics and fabric crosslinked by the method of the prior art.

#### EXAMPLE 2

##### Evaluation of Solvents

Cotton fabrics were prepared (using the method of Example 1) and immersed in solutions of tung oil, pad-

60 Cotton fabrics were prepared (using the method of Example 1) and immersed in solutions of tung oil and acrylonitrile in N,N-dimethylformamide, padded, and dried (using the method of Example 1). Then samples of the dried, tung oil - acrylonitrile treated cotton fabric were cured at 300°F for 6 minutes. Then these cured samples were irradiated with gamma-radiation from cobalt-60 to desired dosages. Selected durable-press properties of the fabrics were determined and are tabulated below. The control fabrics were the same as those in Example 1.

#### EXAMPLE 3

##### Tung Oil, Acrylonitrile, Heat and Radiation:

Cotton fabrics were prepared (using the method of Example 1) and immersed in solutions of tung oil and acrylonitrile in N,N-dimethylformamide, padded, and dried (using the method of Example 1). Then samples of the dried, tung oil - acrylonitrile treated cotton fabric were cured at 300°F for 6 minutes. Then these cured samples were irradiated with gamma-radiation from cobalt-60 to desired dosages. Selected durable-press properties of the fabrics were determined and are tabulated below. The control fabrics were the same as those in Example 1.

TABLE III

Effects of Added Acrylonitrile and Radiation Dosage on the Properties of Tung Oil Cotton Fabrics

| Sample No. | Ratio in Parts of Tung Oil to Monomer | Add-On, % | Radiation Dosage, megarad | Tear Strength, grams | Flex Abrasion Resistance, cycles | Wrinkle Recovery Angle-Wet, degrees |
|------------|---------------------------------------|-----------|---------------------------|----------------------|----------------------------------|-------------------------------------|
| 15         | 7:1                                   | 36        | 2                         | 393                  | 713                              | 256                                 |
| 16         | 3:1                                   | 47        | 2.3                       | 320                  | 587                              | 257                                 |
| 17         | 3:1                                   | 29        | 1.8                       | 460                  | 858                              | 275                                 |
| 18         | 3:1                                   | 23        | 1.1                       | 553                  | 1180                             | 267                                 |
| 19         | 1:1                                   | 33        | 2                         | 320                  | 496                              | 251                                 |

Cotton fabric crosslinked by the method of the prior art (see control fabrics of Example 1) had wrinkle recovery angle-wet of 277°, tear strength of 207 grams, and flex abrasion resistances of 13 cycles, as compared with fabrics prepared by method of Example 3 of 251°-275°, 320-353 grams, and 496-1180 cycles. Obviously, the overall durable-press properties of fabrics prepared by the method of Example 3 were improved over those of fabric prepared by the method of the prior art (see Table III).

#### EXAMPLE 4

##### Evaluation of Monomers

Cotton fabrics were prepared (using the method of Example 1) and immersed in solutions of tung oil and vinyl monomer (10-30%) (acrylonitrile, styrene, diacetone acrylamide, glycidyl methacrylate, or 1,3-butylenedimethacrylate) in N,N-dimethylformamide (80 volume-%) plus methyl ethyl ketone (20 volume-%), padded to wet pickups of 50-250% to yield add-ons of 15 to 68%, and dried (using the method of Example 1). Then samples of the dried, tung oil — vinyl monomer treated cotton fabric were cured at 300° F. for 6 minutes. Then these cured samples were irradiated with gamma-radiation from cobalt-60 to a dosage of 1 megarad. Some of these samples were immersed in hydrazine solution for 17 hours, as indicated in the tabulation below, to improve the odor of the fabrics. Selected durable-press properties of the fabrics were determined and are tabulated below. The control fabrics were the same as those in Example 1.

over those of fabric prepared by the method of the prior art (see Table IV).

We claim:

1. A process for imparting to cotton fabrics improved durable-press properties, the process comprising:
  - a. impregnating a cotton fabric with a 10-30% solution of tung oil in an organic solvent selected from the group consisting of N,N-dimethylformamide, methyl ethyl ketone, a 50-50 mixture of N,N-dimethylformamide and acetone, and a 50-50 mixture of N,N-dimethylformamide and petroleum ether, to a wet pickup of about from 80 to 120%,
  - b. drying the impregnated fabric of (a) with heat applied at about 140°F. for about 3 minutes,
  - c. curing the dried fabric at about from 200° to 300°F. for about from 2 to 8 minutes,
  - d. washing the cured fabric in organic solvent selected from the group consisting of N,N-dimethylformamide, methyl ethyl ketone, or a mixture thereof, and
  - e. drying the cured and washed cotton-tung oil fabric thus produced.
2. The process of claim 1 wherein the organic solvent is N,N-dimethylformamide.
3. The process of claim 1 wherein the organic solvent is methyl ethyl ketone.
4. The process of claim 1 wherein the organic solvent is a 50-50 mixture of N,N-dimethylformamide and acetone.
5. The process of claim 1 wherein the organic solvent is a 50-50 mixture of N,N-dimethylformamide and

TABLE IV

Effects of Monomer Addition and Thermal Plus Radiation Curing on the Properties of Tung Oil Cotton Fabrics

| Sample No. | Monomer <sup>a</sup> | Ratio in Parts of Tung Oil to Monomer | Add-On, % | Tear Strength, grams | Flex Abrasion Resistance, cycles | Wrinkle Recovery Angle-Wet, degrees |
|------------|----------------------|---------------------------------------|-----------|----------------------|----------------------------------|-------------------------------------|
| 20         | AN <sup>b</sup>      | 2.5:1                                 | 15        | 620                  | 924                              | 240                                 |
| 21         | AN                   | 2.5:1                                 | 36        | 460                  | 1066                             | 254                                 |
| 22         | St <sup>b</sup>      | 2.5:1                                 | 32        | 573                  | 1456                             | 252                                 |
| 23         | St                   | 2.5:1                                 | 39        | 420                  | 1067                             | 253                                 |
| 24         | DAA <sup>b</sup>     | 1.3:1                                 | 38        | 433                  | 474                              | 259                                 |
| 25         | GMA <sup>b</sup>     | 1.3:1                                 | 68        | 327                  | 390                              | 246                                 |
| 26         | BDMA                 | 2:1                                   | 48        | 100                  | 95                               | 259                                 |

<sup>a</sup> AN = acrylonitrile; St = styrene; DAA = diacetone acrylamide; GMA = glycidyl methacrylate; BDMA = 1,3-butylenedimethacrylate.

<sup>b</sup> Immersed in hydrazine solution.

Cotton fabrics crosslinked by the method of the prior art (see control fabrics of Example 1) had wrinkle recovery angles-wet of 277°, tear strength of 207 grams, and flex abrasion resistances of 13 cycles, as compared with fabrics prepared by method of Example 4 of 240°-259°, 327-620 grams, and 390-1456 cycles. Obviously, the overall durable-press properties of fabrics prepared by the method of Example 4 were improved

petroleum ether.

6. A process for imparting to cotton fabrics improved durable-press properties, the process comprising:
  - a. impregnating a cotton fabric with a 10-30% solution of a mixture of tung oil and a vinyl monomer selected from the group consisting of acrylonitrile, styrene, diacetone acrylamide, glycidyl methacrylate, and 1,3-butylenedimethacrylate, in a ratio in

parts of tung oil to vinyl monomer about from 7:1 to 1:1, respectively; said mixture in an organic solvent selected from the group consisting of N,N-dimethylformamide and an 80-20 (by volume) mixture of N,N-dimethylformamide and methyl ethyl ketone, to obtain a wet pickup of about from 50 to 250% of yield add-ons of 15 to 68%,  
 b. drying the impregnated fabric of (a) with heat applied at about 140°F. for about 3 minutes,  
 c. curing the dried fabric at about 300°F. for about 6 minutes,  
 d. irradiating the cured fabric with gamma-radiation from cobalt-60 to radiation dosages ranging from about 1 to 2.3 megarads at a temperature of about 77°F to obtain a cotton-tung oil-vinyl polymerized fabric,  
 e. washing the irradiated fabric in N,N-dimethylformamide, and

10

15

20

25

30

35

40

45

50

55

60

65

- f. drying the cured, irradiated, and washed cotton-tung oil-vinyl polymerized fabric.
- 7. The process of claim 6 wherein the vinyl monomer is acrylonitrile.
- 8. The process of claim 6 wherein the vinyl monomer is styrene.
- 9. The process of claim 6 wherein the vinyl monomer is diacetone acrylamide.
- 10. The process of claim 6 wherein the vinyl monomer is glycidyl methacrylate.
- 11. The process of claim 6 wherein the vinyl monomer is 1,3-butylene dimethacrylate.
- 12. The process of claim 6 wherein the organic solvent is N,N-dimethylformamide.
- 13. The process of claim 6 wherein the organic solvent is an 80-20 mixture of N,N-dimethylformamide and methyl ethyl ketone.

\* \* \* \* \*